

Aug. 3, 1943.

J. J. BROPHY

2,325,656

REINFORCING SHOE PARTS

Filed Nov. 28, 1940



INVENTOR  
John J. Brophy  
By his attorney  
Victor Gold

## UNITED STATES PATENT OFFICE

2,325,656

## REINFORCING SHOE PARTS

John J. Brophy, Salem, Mass., assignor to United Shoe Machinery Corporation, Flemington, N. J., a corporation of New Jersey

Application November 28, 1940, Serial No. 367,493

## 1 Claim. (Cl. 12—146)

This invention relates to the reinforcing of uppers of shoes, and is herein illustrated in connection with the reinforcing of a back seam.

In the manufacture of shoes it is common to superpose one quarter upon another with their display faces in contact, and to sew the two quarters together by a seam which lies close to their rear edges, this seam being the back seam of the upper. When the quarters thus sewed together are opened away from each other and turned right side out into the approximate position which they will occupy in the finished shoe, the ends of the quarters beyond the seam form a ridge which projects from the inner faces of the quarters toward what will be the interior of the finished shoe. In order to reduce this ridge and to reinforce the seam, it is common, while the quarters are wrong side out, to separate the two parts of the seam ridge, to bend them apart, to apply pressure to them so as to flatten the ridge, and then to apply to the seam ridge and fasten in place a reinforcing strip of fabric.

The general object of the present invention is to do away with the necessity of providing a preformed reinforcing strip, as well as with the machine which it is necessary to use in applying such a strip to the shoe upper, and at the same time to provide a more effective and more flexible reinforcement.

According to the present invention, an upper is strengthened in a selected locality by applying reinforcing material in flowable form to the locality and causing the material to harden into a tough, flexible reinforcement, which is thus formed in situ. Where such a procedure is followed for the purpose of reinforcing a back seam having a seam ridge, the flowable material may, in some cases, be applied in such manner that it not only covers the seam ridge but substantially fills the hollows on either side of said ridge, thereby obviating the necessity of pressing the seam.

Referring to the accompanying drawing,

Fig. 1 is a perspective showing the application of flowable reinforcing material over the seam ridge and adjacent localities on the inner faces of portions of the quarters which form the rear part of a shoe upper;

Fig. 2 is a cross section of a portion of the rear part of the upper right side out with a reinforcement extending over the seam ridge; and

Fig. 3 is a cross section, similar to that of Fig. 2, showing a seam ridge which has not been pressed, and a reinforcement which not only extends over

the seam ridge but fills the hollows on either side of it.

The shoe part of Fig. 1 consists of two quarters 7 and 9, which have been fastened together by a seam 11, and the seam ridge 13 pressed. In order to strengthen this seam, there is applied, in flowable form over the seam ridge and the adjacent portions of the quarters, a reinforcing material 15 which, upon standing or upon being heated, or both, will harden into a tough flexible reinforcement which adheres firmly to the upper. The reinforcing material may be applied in any suitable manner, for example by being extruded through a properly shaped orifice or, as shown, by means of a brush 17.

In Fig. 2, the quarters are shown right side out in approximately the position they would occupy in the finished shoe, the material 15 having hardened into a tough, flexible reinforcement. In some instances, depending somewhat upon the height of the seam ridge and the type of shoe being made, the pressing of the seam ridge may be omitted and the reinforcing material applied in such manner and quantity that it not only extends over the seam ridge, but fills the hollows on each side of said ridge, as shown at 21 in Fig. 3.

Preferably, a vinyl resin is used as the reinforcing material, since such a resin has qualities of toughness, strength and flexibility which are particularly desirable, and since a reinforcement in the form of a strip or band of such resin formed in situ adheres very firmly to the shoe part. The following are examples of preparations of vinyl resins which may be used.

## Example I

|                    | Parts by weight |
|--------------------|-----------------|
| Vinylite XYSG      | 18              |
| 40 Plasticiser 3GH | 9               |
| Ethyl alcohol      | 66              |
| Cellosolve         | 7               |

These ingredients are mixed cold to produce a viscous solution which tends to gel upon standing. The viscous solution or gel, heated to about 110° to render it properly flowable, is applied to the shoe part.

## Example II

|                                    | Parts by weight |
|------------------------------------|-----------------|
| Polyvinyl alcohol (high viscosity) | 18              |
| Sorbitol (solid)                   | 10              |
| Water                              | 72              |

The polyvinyl alcohol and the sorbitol are stirred into the water, and then the solution is

heated to 160° F. with further stirring. It may be applied to the shoe part at about that temperature.

Having thus described my invention, what I claim as new and desire to secure by Letters Patent of the United States is:

The method of reinforcing the back seam joining the quarters which form the rear portion of the upper of a shoe prior to incorporating the rear portion in a shoe, the back seam having a

10  
10

side of the upper, said method comprising turning the said rear portion of the upper wrong side out to give easy access to the seam ridge, applying over the seam ridge and the closely adjacent portions of the quarters only a reinforcing material in flowable form, and causing the material to solidify into a tough, flexible reinforcement which adheres to the seam ridge and to the adjacent portions of the quarters on each side of said ridge.

JOHN J. BROPHY.